

# United States Patent [19]

Keevert, Jr. et al.

[11] Patent Number: 4,945,035

[45] Date of Patent: \* Jul. 31, 1990

[54] **PHOTOGRAPHIC EMULSIONS  
CONTAINING INTERNALLY MODIFIED  
SILVER HALIDE GRAINS**

[75] Inventors: John E. Keevert, Jr.; Woodrow G. McDugle; Raymond S. Eachus, all of Rochester, N.Y.

[73] Assignee: Eastman Kodak Company, Rochester, N.Y.

[\*] Notice: The portion of the term of this patent subsequent to May 20, 2006 has been disclaimed.

[21] Appl. No.: 179,377

[22] Filed: Apr. 8, 1988

[51] Int. Cl.<sup>5</sup> ..... G03C 1/06

[52] U.S. Cl. ..... 430/567; 430/569; 430/596; 430/604; 430/605; 430/606; 430/612

[58] Field of Search ..... 430/567, 569, 604, 605, 430/606, 612, 596

[56] **References Cited**

**U.S. PATENT DOCUMENTS**

|           |         |                  |       |         |
|-----------|---------|------------------|-------|---------|
| 2,448,060 | 8/1948  | Trivelli et al.  | ..... | 430/603 |
| 3,790,390 | 2/1974  | Shiba et al.     | ..... | 430/567 |
| 3,890,154 | 6/1975  | Ohkubo           | ..... | 430/434 |
| 4,126,472 | 11/1978 | Sakai et al.     | ..... | 430/264 |
| 4,147,542 | 4/1979  | Habu             | ..... | 430/346 |
| 4,643,965 | 2/1987  | Kubot et al.     | ..... | 430/567 |
| 4,835,093 | 5/1989  | Janusonig et al. | ..... | 430/567 |

**FOREIGN PATENT DOCUMENTS**

|            |         |                    |               |
|------------|---------|--------------------|---------------|
| 0242190/A2 | 10/1987 | European Pat. Off. | .....         |
| 62-212641  | 9/1987  | Japan              | ..... 430/605 |

**OTHER PUBLICATIONS**

*Research Disclosure*, vol. 176, Dec. 1978, Item 17643, Section IA.

D. M. Samoilovich, "The Influence of Rhodium and Other Polyvalent Ions on the Photographic Properties of Silver Halide Emulsions", in a paper presented to 1978 International Congress of Photographic Science, Rochester Institute of Technology, Aug. 20-26, 1978. At the 1982 International Congress of Photographic Science at the University of Cambridge, R. S. Eachus presented a paper titled, "The Mechanism of Ir<sup>3+</sup> Sensitization of Silver Halide Materials".

B. H. Carroll, "Iridium Sensitization: A Literature Review", *Photographic Science and Engineering*, vol. 24, No. 6, Nov./Dec. 1980, pp. 265-267, is cited for further background on the use of iridium in silver halide emulsions.

Primary Examiner—Roland E. Martin

Assistant Examiner—Janet C. Baxter

Attorney, Agent, or Firm—Carl O. Thomas

[57] **ABSTRACT**

Photographic silver halide emulsions are disclosed comprised of radiation sensitive silver halide grains containing greater than 50 mole percent chloride and less than 5 mole percent iodide, based on total silver, with any residual halide being bromide, said grains exhibiting a face centered cubic crystal lattice structure formed in the presence of a hexacoordination complex of rhenium, ruthenium, or osmium with at least four cyanide ligands. The emulsions exhibit increased sensitivity.

14 Claims, 1 Drawing Sheet



FIG. 1

PHOTOGRAPHIC EMULSIONS CONTAINING  
INTERNAL MODIFIED SILVER HALIDE  
GRAINS

FIELD OF THE INVENTION

The invention relates to photography. More specifically, the invention relates to photographic silver halide emulsions and to photographic elements containing these emulsions.

DEFINITION OF TERMS

All references to periods and groups within the periodic table of elements are based on the format of the periodic table adopted by the American Chemical Society and published in the *Chemical and Engineering News*, Feb. 4, 1985, p. 26. In this form the prior numbering of the periods was retained, but the Roman numeral numbering of groups and designations of A and B groups (having opposite meanings in the U.S. and Europe) was replaced by a simple left to right 1 through 18 numbering of the groups.

The term "high chloride emulsion" refers to a silver halide emulsion which contains greater than 50 mole percent chloride and less than 5 mole percent iodide, based on total silver, with any remaining halide being bromide.

The term "dopant" refers to a material other than a silver or halide ion contained within a silver halide grain.

The term "transition metal" refers to any element of groups 3 to 12 inclusive of the periodic table of elements.

The term "heavy transition metal" refers to transition metals of periods 5 and 6 of the periodic table of elements.

The term "light transition metal" refers to transition metals of period 4 of the periodic table of elements.

The term "palladium triad transition metals" refers to period 5 elements in groups 8 to 10 inclusive—i.e., ruthenium, rhodium, and palladium.

The term "platinum triad transition metals" refers to period 6 elements in groups 8 to 10 inclusive—i.e., osmium, iridium, and platinum.

The acronym "EPR" refers to electron paramagnetic resonance.

The acronym "ESR" refers to electron spin resonance.

The term "pK<sub>sp</sub>" indicates the negative logarithm of the ty product constant of a compound.

Grain sizes, unless otherwise indicated, are mean effective circular diameters of the grains, where the effective circular diameter is the diameter of a circle having an area equal to the projected area of the grain.

Photographic speeds are reported as relative speeds, except as otherwise indicated.

PRIOR ART

Trivelli and Smith U.S. Pat. No. 2,448,060, issued Aug. 31, 1948, taught that silver halide emulsions can be sensitized by adding to the emulsion at any stage of preparation—i.e., before or during precipitation of the silver halide grains, before or during the first digestion (physical ripening), before or during the second digestion (chemical ripening), or just before coating, a compound of a palladium or platinum triad transition metal, identified by the general formula:

$R_2MX_6$   
wherein

5 R represents a hydrogen atom, an alkali metal atom, or an ammonium radical,

M represents a palladium or platinum triad transition metal, and

X represents a halogen atom—e.g., a chlorine or bromine atom.

10 The formula compounds are hexacoordinated heavy transition metal complexes which are water soluble. When dissolved in water R<sub>2</sub> dissociates as two cations while the transition metal and halogen ligands disperse as a hexacoordinated anionic complex.

15 With further investigation the art has recognized a distinct difference in the photographic effect of transition metal compounds in silver halide emulsions, depending upon whether the compound is introduced into the emulsion during precipitation of silver halide grains or subsequently in the emulsion making process. In the former instance it has been generally accepted that the transition metal can enter the silver halide grain as a dopant and therefore be effective to modify photographic properties, though present in very small concentrations.

20 Then transition metal compounds are introduced into an emulsion after silver halide grain precipitation is complete, the transition metals can be absorbed to the grain surfaces, but are sometimes largely precluded from grain contact by peptizer interactions. Orders of magnitude higher concentrations of transition metals are required to show threshold photographic effects when added following silver halide grain formation as compared to transition metals incorporated in silver halide grains as dopants. The art distinction between metal doping, resulting from transition metal compound addition during silver halide grain formation, and transition metal sensitizers, resulting from transition metal compound addition following silver halide grain formation, is illustrated by *Research Disclosure*

30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655

palladium and platinum triad transition metal and the remainder of the compound is provided by other than halide ligands, halide and aquo ligands, halides which dissociate to form anions in solution, or ammonium or alkali metal moieties that dissociate to form cations in solution. The following is a listing of the few variant teachings that have been identified:

Shiba et al U.S. Pat. No. 3,790,390 discloses preparing a blue responsive silver halide emulsion suitable for flash exposure which can be handled under bright yellowish-green light. The emulsion contains grains with a mean size no larger than 0.9  $\mu\text{m}$ , at least one group 8-10 metal compound, and a formula specified merocyanine dye. Examples of transition metal compounds are simple salts of light transition metals, such as iron, cobalt, and nickel salts, and hexacoordinated complexes of light transition metals containing cyano ligands. Significantly, there is no teaching or suggestion of employing cyano ligands with heavy transition metals. Heavy transition metal compounds are disclosed only as the usual simple salts or hexacoordinated complexes containing only halide ligands. Palladium (II) nitrate, a simple salt, is also disclosed as well as palladium tetrathiocyanatopalladate (II), a tetracoordinated complex of palladium.

Ohkubo et al U.S. Pat. No. 3,890,154 and Habu et al U.S. Pat. No. 4,147,542 are similar to Shiba et al, differing principally in employing different sensitizing dyes to allow recording of green flash exposures.

Sakai et al U.S. Pat. No. 4,126,472 discloses producing a high contrast emulsion suitable for lith photography by ripening an emulsion containing at least 60 mole percent silver chloride in the presence of  $10^{-6}$  to  $10^{-4}$  mole per mole of silver halide of a water soluble iridium salt and further adding a hydroxytetraazaindene and a polyoxyethylene compound. In addition to the usual iridium halide salts and hexacoordinated iridium complexes containing halide ligands Sakai et al discloses cationic hexacoordinated complexes of iridium containing amine ligands. Since iridium is introduced after silver halide precipitation is terminated, the iridium is not employed as a grain dopant, but as a grain surface modifier. This undoubtedly accounts for the variance from conventional iridium compounds used for doping.

D.M. Samoilovich, "The Influence of Rhodium and Other polyvalent Ions on the photographic properties of Silver Halide Emulsions", in a paper presented to 1978 International Congress of photographic Science, Rochester Institute of Technology, Aug 20-26, 1978, reported investigations of chloride iridium, rhodium, and gold complexes and, in addition, an emulsion prepared by introducing  $(\text{NH}_4)_6\text{Mo}_7\text{O}_{24}\text{H}_2\text{O}$ . The latter dissociates in water form a molybdenum cluster having a net negative charge of -6. Neither the +6 oxidation state ascribed to molybdenum nor the -6 valence of the anionic cluster should be confused with a hexacoordinated complex of a single transition metal atom.

At the 1982 International Congress of photographic Science at the University of Cambridge, R. S. Eachus presented a paper titled, "The Mechanism of  $\text{Ir}^{3+}$  Sensitization of Silver Halide Materials", wherein inferential electron paramagnetic resonance (EPR) spectroscopic evidence was presented that  $\text{Ir}^{3+}$  ions were incorporated into melt grown silver bromide and silver chloride crystals as  $(\text{IrBr}_6)^{-3}$  and  $(\text{IrCl}_6)^{-3}$ . In emulsions and sols of these salts, the hexabromoiridate and hexachloroiridate molecular ions, as well as similar complexes containing mixed halides, were introduced during precipitation. The aquated spe-

cies  $[\text{IrCl}_4(\text{H}_2\text{O})_2]^{-1}$  and  $[\text{IrCl}_5(\text{H}_2\text{O})]^{-2}$  were also successfully doped into precipitates of both silver salts. Eachus went on to speculate on various mechanisms by which incorporated iridium ions might contribute to photogenerated free electron and hole management, including latent image formation. B. H. Carroll, "Iridium Sensitization: A Literature Review", *Photographic Science and Engineering*, Vol. 24, No. 6, Nov./Dec. 1980, pp. 265-267, is cited for further background.

Greskowiak Published European Patent Application No. 0,242,90/ A2 discloses reductions in high intensity reciprocity failure in silver halide emulsions formed in the presence of one or more complex compounds of rhodium (III) having 3, 4, 5, or 6 cyanide ligands attached to each rhodium ion.

#### RELATED PATENT APPLICATIONS

McDugle et al U.S. Ser. No. 179,376 filed concurrently herewith and commonly assigned, titled PHOTOGRAPHIC EMULSIONS CONTAINING INTERNALLY MODIFIED SILVER HALIDE GRAINS, discloses silver halide emulsions comprised of radiation sensitive silver halide grains exhibiting a face centered cubic crystal lattice structure internally containing a nitrosyl or thionitrosyl coordination ligand and a transition metal chosen from groups 5 to 10 inclusive of the periodic table of elements.

Marchetti et al U.S. Ser. No. 179,378, concurrently filed and commonly assigned, titled PHOTOGRAPHIC EMULSIONS CONTAINING INTERNALLY MODIFIED SILVER HALIDE GRAINS, discloses photographic emulsions comprised of radiation sensitive silver bromide or bromoiodide grains which exhibit a face centered cubic crystal structure formed in the presence of a hexacoordination complex of rhenium, ruthenium, or osmium with at least four cyanide ligands.

Janusonis et al, U.S. Ser. No. 179,380, concurrently filed and commonly assigned, titled INTERNALLY DOPED SILVER HALIDE EMULSIONS, now U.S. Pat. No. 4,835,093 discloses photographic emulsions comprised of silver halide grains exhibiting a face centered cubic crystal lattice structure and internally containing rhenium.

#### SUMMARY OF THE INVENTION

In one aspect this invention is directed to a photographic silver halide emulsion comprised of radiation sensitive silver halide grains containing greater than 50 mole percent chloride and less than 5 mole percent iodide, based on total silver, with any residual halide being bromide, said grains exhibiting a face centered cubic crystal lattice structure formed in the presence of a hexacoordination complex of rhenium, ruthenium, or osmium with at least four cyanide ligands.

Surprisingly, increased sensitivities are produced in high chloride emulsions formed in the presence of these rhenium, ruthenium, and osmium coordination complexes. Whereas, when another transition metal is substituted, either no sensitization or desensitization has been observed. Additionally, when rhenium, ruthenium, or osmium coordination complexes containing ligands other than the required cyanide ligands, the photographic effect is not observed.

## BRIEF DESCRIPTION OF THE DRAWINGS

FIG. 1 is a schematic view of a silver bromide crystal structure with the upper layer of ions lying along a {100} crystallographic face.

## DESCRIPTION OF PREFERRED EMBODIMENTS

The present invention is directed to high chloride emulsions which exhibit increased sensitivity. Such emulsions contain greater than 50 mole percent (preferably greater than 70 mole percent and optimally greater than 85 mole percent) chloride. The emulsions contain less than 5 mole percent iodide (preferably less than 2 mole percent) iodide, with the balance, if any, of the halide being iodide.

It has been discovered quite unexpectedly that the sensitivity of these emulsions can be increased when the grains of the emulsion are formed in the presence of a hexacoordination complex of rhenium, ruthenium, or osmium with at least four cyanide ligands. Surprisingly, sensitization has not been observed when other transition metals (more specifically identified in the examples below) have been substituted for rhenium, ruthenium, or osmium. Further, it has been observed that sensitization is not achieved when the cyanide ligands are replaced with other ligands. This latter observation suggests that both the transition metal and cyanide ligands are incorporated in the grains as they are being formed.

It is in fact believed that the entire hexacoordinated transition metal complex is incorporated intact in the grains being formed. To understand how this can be possible, it is helpful to first review the structure of silver halide grains. Unlike silver iodide, which commonly forms only  $\beta$  and  $\gamma$  phases and is rarely used in photography, each of silver chloride and silver bromide form a face centered cubic crystal lattice structure of the rock salt type. In FIG. 1 four lattice planes of a crystal structure 1 of silver ions 2 and bromide ions 3 is shown, where the upper layer of ions lies in a {100} crystallographic plane. The four rows of atoms shown counting from the bottom of FIG. 1 lie in a {100} crystallographic plane which perpendicularly intersects the [100] crystallographic plane occupied by the upper layer of ions. The row containing silver ions 2a and bromide ions 3a lies in both intersecting planes. In each of the two {100} crystallographic planes it can be seen that each silver ion and each bromide ion lies next adjacent to four bromide ions and four silver ions, respectively. In three dimensions then, each interior silver ion lies next adjacent to six bromide ions, four in the same {100} crystallographic plane and one on each side of the plane. A comparable relationship exists for each interior bromide ion.

The arrangement of atoms in a silver chloride crystal is the same as that shown in FIG. 1, except that chloride ions are smaller than bromide ions. Silver halide grains in photographic emulsions can be formed of bromide ions as the sole halide, chloride ions as the sole halide, or any mixture of the two. It is also common practice to incorporate minor amounts of iodide ions in photographic silver halide grains. Since chlorine, bromine, and iodine are 3rd, 4th, and 5th period elements, respectively, the iodide ions are larger than the bromide ions.

The manner in which a hexacoordinated transition metal complex can be incorporated in the grain structure can be roughly appreciated by considering the characteristics of a single silver ion and six adjacent

halide ions (hereinafter collectively referred to as the seven vacancy ions) that must be omitted from the crystal structure to accommodate spatially the hexacoordinated transition metal complex. The seven vacancy ions exhibit a net charge of -5. This suggests that anionic transition metal complexes should be more readily incorporated in the crystal structure than neutral or cationic transition metal complexes. This also suggests that the capability of a hexacoordinated heavy transition metal complex to trap either photogenerated holes or electrons may be determined to a significant degree by whether the complex introduced has a net charge more or less negative than the seven vacancy ions it displaces. This is an important departure from the common view that heavy transition metals are incorporated into silver halide grains as bare ions or atoms and that their hole or electron trapping capability is entirely a function of their oxidation state.

Referring to FIG. 1, it should be further noted that the silver ions are much smaller than the bromide ions, though silver lies in the 5th period while bromine lies in the 4th period. Further, the lattice is known to accommodate iodide ions, which are still larger than bromide ions. This suggests that the size of 5th and 6th period transition metals should not in itself provide any barrier to their incorporation. A final observation that can be drawn from the seven vacancy ions is that the six halide ions exhibit an ionic attraction not only to the single silver ion that forms the center of the vacancy ion group, but are also attracted to other adjacent silver ions.

Hexacoordinated complexes exhibit a spatial configuration that is compatible with the face centered cubic crystal structure of photographically useful silver halides. The six ligands are spatially comparable to the six halide ions next adjacent to a silver ion in the crystal structure. To appreciate that a hexacoordinated complex of a heavy transition metal having ligands other than halide ligands or, as recognized by Eachus, cited above, aquo ligands, can be accommodated into silver halide cubic crystal lattice structure it is necessary to consider that the attraction between the transition metal and its ligands is not ionic, but the result of covalent bonding, the latter being much stronger than the former. Since the size of a hexacoordinated complex is determined not only by the size of the atoms forming the complex, but also by the strength of the bonds between the atoms, a hexacoordinated complex can be spatially accommodated into a silver halide crystal structure in the space that would otherwise be occupied by the seven vacancy ions, even though the number and/or diameters of the individual atoms forming the complex exceeds that of the vacancy ions. This is because the covalent bond strength can significantly reduce bond distances and therefore the size of the entire complex. It is a specific recognition of this invention that multielement ligands of hexacoordinated transition metal complexes can be spatially accommodated to single halide ion vacancies within the crystal structure.

While spatial compatibility is important in choosing suitable hexacoordinated transition metal complexes, another factor which must be taken into account is the compatibility of the complex with the next adjacent ions in the crystal lattice structure. It is the recognition of this invention that compatibility can be realized by choosing bridging ligands for the transition metal complex. Looking at a single row of silver and halide ions in

a cubic crystal lattice structure, the following relationship can be observed:



Notice that the halide ions X are attracting both adjacent silver ions in the row. When the portion of a hexacoordinated transition metal complex lying in a single row of silver and halide ions in a crystal structure is considered, the following relationship can be observed:



where

M represents a heavy transition metal and

L represents a bridging ligand.

While only one row of silver and halide ions is shown, it is appreciated that the complex forms part of three identical perpendicular rows of silver and halide ions having the heavy transition metal M as their point of intersection. However, since the three rows are identical, the relationships can be appreciated from considering a single row.

Transition metal coordination complexes satisfying the requirements of this invention are those which contain rhenium, ruthenium, or osmium as a transition metal and 4, 5, or 6 cyanide ligands. When only 4 or 5 cyanide ligands are present, the remaining ligands or ligand can be any convenient conventional bridging ligand. The latter when incorporated in the silver halide crystal structure are capable of serving as bridging groups between two or more metal centers. These bridging ligands can be either monodentate or ambidentate. A monodentate bridging ligand has only one ligand atom that forms two (or more) bonds to two (or more) different metal atoms. For monoatomic ligands and for those containing only one donor atom, only the monodentate form of bridging is possible. Multielement ligands with more than one donor atom can also function in a bridging capacity and are referred to as ambidentate ligands. Preferred bridging ligands are monoatomic monodentate ligands, such as halides. Fluoride, chloride, bromide, and iodide ligands are all specifically contemplated. Multielement ligands, such as azide and thiocyanate ligands, are also specifically contemplated.

The hexacoordinated rhenium, ruthenium, and osmium cyanide complexes contemplated for grain incorporation in most instances exhibit a net ionic charge. One or more counter ions are therefore usually associated with the complex to form a charge neutral compound. The counter ion is of little importance, since the complex and its counter ion or ions dissociate upon introduction into an aqueous medium, such as that employed for silver halide grain formation. Ammonium and alkali metal counterions are particularly suitable for anionic hexacoordinated complexes satisfying the requirements of this invention, since these cations are known to be fully compatible with silver halide precipitation procedures.

In a preferred form the hexacoordinated rhenium, ruthenium, and osmium cyanide complexes can be represented by the following formula:



(I)

where

M is rhenium, ruthenium, or osmium,

L is a bridging ligand,

y is the integer zero, 1, or, 2, and

-n is -2, -3, or -4

Table I provides a listing of illustrative rhenium, ruthenium, and osmium cyanide coordination complexes satisfying the requirements of the invention:

TABLE I

|        |                                                     |
|--------|-----------------------------------------------------|
| TMC-1  | $[\text{Re}(\text{CN})_6]^{-4}$                     |
| TMC-2  | $[\text{Ru}(\text{CN})_6]^{-4}$                     |
| TMC-3  | $[\text{Os}(\text{CN})_6]^{-4}$                     |
| TMC-4  | $[\text{ReF}(\text{CN})_5]^{-4}$                    |
| TMC-5  | $[\text{RuF}(\text{CN})_5]^{-4}$                    |
| TMC-6  | $[\text{OsF}(\text{CN})_5]^{-4}$                    |
| TMC-7  | $[\text{ReCl}(\text{CN})_5]^{-4}$                   |
| TMC-8  | $[\text{RuCl}(\text{CN})_5]^{-4}$                   |
| TMC-9  | $[\text{OsCl}(\text{CN})_5]^{-4}$                   |
| TMC-10 | $[\text{ReBr}(\text{CN})_5]^{-4}$                   |
| TMC-11 | $[\text{RuBr}(\text{CN})_5]^{-4}$                   |
| TMC-12 | $[\text{OsBr}(\text{CN})_5]^{-4}$                   |
| TMC-13 | $[\text{ReI}(\text{CN})_5]^{-4}$                    |
| TMC-14 | $[\text{RuI}(\text{CN})_5]^{-4}$                    |
| TMC-15 | $[\text{OsI}(\text{CN})_5]^{-4}$                    |
| TMC-16 | $[\text{ReF}_2(\text{CN})_4]^{-4}$                  |
| TMC-17 | $[\text{RuF}_2(\text{CN})_4]^{-4}$                  |
| TMC-18 | $[\text{OsF}_2(\text{CN})_4]^{-4}$                  |
| TMC-19 | $[\text{ReCl}_2(\text{CN})_4]^{-4}$                 |
| TMC-20 | $[\text{RuCl}_2(\text{CN})_4]^{-4}$                 |
| TMC-21 | $[\text{OsCl}_2(\text{CN})_4]^{-4}$                 |
| TMC-22 | $[\text{RuBr}_2(\text{CN})_4]^{-4}$                 |
| TMC-23 | $[\text{OsBr}_2(\text{CN})_4]^{-4}$                 |
| TMC-24 | $[\text{ReBr}_2(\text{CN})_4]^{-4}$                 |
| TMC-25 | $[\text{RuI}_2(\text{CN})_4]^{-4}$                  |
| TMC-26 | $[\text{OsI}_2(\text{CN})_4]^{-4}$                  |
| TMC-27 | $[\text{Ru}(\text{CN})_5(\text{OCN})]^{-4}$         |
| TMC-28 | $[\text{Os}(\text{CN})_5(\text{OCN})]^{-4}$         |
| TMC-29 | $[\text{Ru}(\text{CN})_5(\text{SCN})]^{-4}$         |
| TMC-30 | $[\text{Os}(\text{CN})_5(\text{SCN})]^{-4}$         |
| TMC-31 | $[\text{Ru}(\text{CN})_5(\text{N}_3)]^{-4}$         |
| TMC-32 | $[\text{Os}(\text{CN})_5(\text{N}_3)]^{-3}$         |
| TMC-33 | $[\text{Ru}(\text{CN})_5(\text{H}_2\text{O})]^{-3}$ |
| TMC-34 | $[\text{Os}(\text{CN})_5(\text{H}_2\text{O})]^{-3}$ |

Procedures for beginning with the compounds of Table I and preparing photographic silver halide emulsions benefitted by incorporation of the hexacoordinated rhenium, ruthenium, or osmium cyanide complex can be readily appreciated by considering the prior teachings of the art relating to introducing heavy transition metal dopants in silver halide grains. Such teachings are illustrated by Wark U.S. Pat. No. 2,717,833; Berriman U.S. Pat. No. 3,367,778; Burt U.S. Pat. No. 3,445,235; Bacon et al U.S. Pat. No. 3,446,927; Colt U.S. Pat. No. 3,418,122; Bacon U.S. Pat. No. 3,531,291; Bacon U.S. Pat. No. 3,574,625; Japanese Patent (Kokoku) No. 33781/74 (Priority 10 May 1968); Japanese Patent (Kokoku) No. 30483/73 (priority 2 Nov. 1968); Ohkubo et al U.S. Pat. No. 3,890,154; Spence et al U.S. Pat. Nos. 3,687,676 and 3,690,891; Gilman et al U.S. Pat. No. 3,979,213; Motter U.S. Pat. No. 3,703,584; Japanese Patent (Kokoku) No. 32738/70 (priority 22 Oct. 1970); Shiba et al U.S. Pat. No. 3,790,390; Yamasue et al U.S. Pat. No. 3,901,713; Nishina et al U.S. Pat. No. 3,847,621; *Research Disclosure*, Vol. 108, Apr. 1973, Item 10801; Sakai U.S. Pat. No. 4,126,472; Dostes et al Defensive Publication No. T962,004 and French Patent No. 2,296,204; U.K. Specification No. 1,527,435 (priority 17 Mar. 1975); Japanese Patent Publication (Kokai) No. 107,129/76 (priority 18 Mar. 1975); Habu et al U.S. Pat. Nos. 4,147,542 and 4,173,483; *Research Disclosure*, Vol. 134, June 1975, Item 13452; Japanese Patent Publication (Kokai) No. 65,432/77 (priority 26 Nov. 1975); Japanese Patent Publication (Kokai) No. 76,923/77 (priority 23 Dec. 1975); Japanese Patent Publication (Kokai) No. 88,340/77 (priority 26 Jan. 1976); Japanese Patent Publication (Kokai) No. 75,921/78 (priority 17

Dec. 1976); Okutsu et al U.S. Pat. No. 4,221,857; Japanese Patent Publication (Kokai) No. 96,024/79 (priority 11 Jan. 1978); *Research Disclosure*, Vol. 181, May 1979, Item 18155; Kanisawa et al U.S. Pat. No. 4,288,533; Japanese Patent Publication (Kokai) No. 25,727/81 (Priority 7 Aug. 1979); Japanese Patent Publication (Kokai) 51,733/81 (priority 2 Oct. 1979); Japanese Patent Publication (Kokai) No. 166,637/80 (priority 6 Dec. 1979); and Japanese Patent Publication (Kokai) No. 149,142/81 (priority 18 Apr. 1970); the disclosures of which are here incorporated by reference.

When silver halide grains are formed a soluble silver salt, usually silver nitrate, and one or more soluble halide salts, usually an ammonium or alkali metal halide salt, are brought together in an aqueous medium. Precipitation of silver halide is driven by the high  $pK_{sp}$  of silver halides, ranging from 9.75 for silver to 16.09 for silver iodide at room temperature. For the rhenium, ruthenium, or osmium cyanide complex to coprecipitate with silver halide it must also form a high  $pK_{sp}$  compound. If the  $pK_{sp}$  is too low, precipitation may not occur. On the other hand, if the  $pK_{sp}$  is too high, the compound may precipitate as a separate phase. Optimum  $pK_{sp}$  values for silver counter ion compounds of rhenium, ruthenium, or osmium cyanide complexes contemplated for use in the practice of this invention are in or near the range of  $pK_{sp}$  values for photographic silver halides—that is, in the range of from about 8 to 20, preferably about 9 to 17.

Apart from the incorporated hexacoordinated heavy transition metal complexes satisfying the requirements of the invention the silver halide grains, the emulsions of which they form a part, and the photographic elements in which they are incorporated can take any of a wide variety of conventional forms. A survey of these conventional features as well as a listing of the patents and publications particularly relevant to each teaching is provided by *Research Disclosure*. Item 17643, cited above, the disclosure of which is here incorporated by reference. It is specifically contemplated to incorporate hexacoordinated heavy transition metal complexes satisfying the requirements of this invention in tabular grain emulsions, particularly thin (less than 0.2  $\mu\text{m}$ ) and/or high aspect ratio ( $>8:1$ ) tabular grain emulsions, such as those disclosed in Kofron et al U.S. Pat. No. 4,439,520; Wey U.S. Pat. No. 4,399,215; Dickerson U.S. Pat. No. 4,414,304; Maskasky U.S. Pat. Nos. 4,400,463, 4,435,501, 4,643,966, and 4,713,320; and Daubendiek et al U.S. Pat. Nos. 4,672,027 and 4,693,964; the disclosures of which are here incorporated by reference.

It has been determined by imagewise exposure, bleaching of surface latent image, and then development in an internal developer, that increased internal sensitivity can be imparted to high chloride emulsions by precipitating the grains in the presence of hexacoordinated rhenium, ruthenium, or osmium cyanide complexes of the type described above. Effective concentrations of the emulsion range from about  $1 \times 10^{-6}$  mole of complex per silver mole. The complex can be incorporated into the grains up to its solubility limit, typically about  $5 \times 10^{-4}$  mole per silver mole. An excess of the complex over its solubility limit in the grain can be tolerated, but normally any such excess is removed from the emulsion during washing. Preferred concentrations of the complex for achieving internal sensitivity are from  $10^{-5}$  to  $10^{-4}$  mole per silver mole.

When increased internal sensitivity is sought, surface competition for photogenerated electrons should be

avoided. Thus, these emulsions are preferably free of intentional surface chemical sensitization. Obtaining increased internal sensitivity is, however, entirely compatible with and can be enhanced by incorporating conventional hole trapping spectral sensitizing dyes in the emulsions.

It has been surprisingly discovered that when the internally sensitized emulsions are further modified by conventional surface sulfur and/or gold sensitization—i.e., whether the sulfur or gold sensitization is the sole sensitizing agent or employed in combination with other conventional sensitizers, the emulsions exhibit increased surface sensitivity as compared to a control emulsion which is identically surface sensitized, but lacks the incorporated complex. Other conventional chalcogen sensitizers can be substituted for sulfur, if desired.

## EXAMPLES

The invention can be better appreciated by reference to the following specific examples:

### EXAMPLE 1

A  $\text{AgCl}$  powder was made without the use of any peptizing agent such as gelatin in which the variation made was in the presence of  $\text{K}_4\text{Os}(\text{CN})_6$  as a dopant.

The solutions were prepared as follows:

| Solution 1/1                    |           |
|---------------------------------|-----------|
| Silver nitrate                  | 33.98 gms |
| Distilled water to total volume | 100 ml    |
| Solution 2/1                    |           |
| Potassium chloride              | 15.66 gms |
| Distilled water to total volume | 100 ml    |

We have incorporated an anionic transition metal complex,  $[\text{Os}(\text{CN})_6]^{4-}$ , into the  $\text{AgCl}$  lattice in the absence of gelatin by adding, in the dark, 100 ml of 2 M  $\text{AgNO}_3$  (Solution 1/1) through one delivery buret and 100 ml of 2.1 M KCl (5% excess) (Solution 1) through a second delivery buret into a common reaction vessel. The  $[\text{Os}(\text{CN})_6]^{4-}$  complex is usually added as the potassium salt. The reaction vessel initially contained 100 ml of water and was preheated to ca. 50° C. The reaction vessel was vigorously stirred during the  $\text{AgNO}_3$  and KCl addition. The temperature in the reaction vessel fell a few degrees below 50° C during the reaction due to the inrush of room temperature reactants. The addition was generally complete in ca. 6 to 7 minutes. The addition rate was controlled manually with the only criteria that the KCl buret addition be equal to or slightly ahead, but by no more than 1 milliliter, of the  $\text{AgNO}_3$  addition. The dopant was added both through a third pipette or through the KCl solution without any noticeable difference occurring between the two addition methods. The dopant was added in a number of individual steps during the entire precipitation when added through a separate pipette and continuously during the entire precipitation when added through the KCl delivery buret along with the KCl. The samples were washed well with water, ca. 500 ml of water for each 0.2 moles of  $\text{AgCl}$  precipitated. The samples were then washed several times with approximately 50 ml of acetone each time and the acetone decanted after each washing, filtered using a #2 qualitative paper filter, washed with diethyl ether, and then stored in open glass dishes in the dark until dry.

ESR of the  $K_4Os(CN)_6$  doped  $AgCl$  sample before any light exposure does not show any paramagnetic osmium species. This is in contrast to the ESR of  $AgCl$  doped with the  $[OsCl_6]^{-3}$  coordination complex, using  $K_2OsCl_6$  as the dopant, which clearly shows paramagnetic centers  $Os^{+3}$  centers present even without light exposure. After exposure of the  $[Os(CN)_6]^{-4}$  doped  $AgCl$  powder samples to 365 nm radiation, ESR shows the presence of paramagnetic  $Os^{+3}$  centers that result from hole paramagnetic  $Os^{+2}$  centers.

The control  $AgCl$  powder without any  $K_4Os(CN)_6$  dopant did not show any ESR spectra, under any conditions, of an osmium center of any type.

#### EXAMPLE 2

A  $AgCl$  powder sample was prepared as described in Example 1 except that both  $K_2Ru(NO)Cl_5$  and  $K_4Os(CN)_6$  were used to co-dope the same sample. ESR of this sample, after exposure to 365 nm radiation, showed that the  $[Ru(NO)Cl_5]^{-2}$  centers were trapping electrons to produce  $[Ru(NO)Cl_5]^{-3}$  centers and that the  $[Os(CN)_6]^{-4}$  centers were trapping holes to produce  $[Os(CN)_6]^{-3}$  centers. The two centers were not competing for the same electronic species, the photoproduced electron or the photoproduced hole. This is completely consistent with Example 1.

#### EXAMPLE 3

##### Emulsion

0.3  $\mu m$  Undoped  $AgCl$  (Control)

At 40° C., 75 g of gelatin was added to 2 liters of water in a reaction vessel and the PH of the reaction vessel contents was adjusted to 3.0. The temperature was raised to 55° C., and the chloride ion concentration was adjusted to 0.041 molar. Concentrated aqueous silver nitrate was pumped into the vigorously stirred gelatin solution along with sufficient aqueous sodium chloride solution to maintain the quoted concentration. A third aqueous solution was introduced into the reaction vessel, starting 3 minutes after introduction of the silver nitrate solution. Precipitation was continued until 6 moles of approximately 0.3  $\mu m$  silver chloride grains were formed.

After washing by the coagulation method of Yutzy and Russell U.S. Pat. No. 2,614,929, a portion of the emulsion was optimally gold sensitized, chilled, and then prepared for coating by the addition of extra gelatin and a spreading agent. Coatings on a cellulose acetate film support were exposed through a step tablet to 365 nm radiation and processed for 5 minutes in a hydroquinone-Elon ®(N methyl-p aminophenol hemisulfate) developer. After fixing and washing the coating, the photographic speed was determined at a density of 0.3 above fog.

##### Emulsion 2

0.3  $\mu m$   $[Os(CN)_6]^{-4}$  Doped  $AgCl$

##### (Example)

The procedure described above in connection with Emulsion 1 was repeated, except that the third aqueous solution contained 69.5 mg  $K_4Os(CN)_6$  to produce a reaction vessel concentration of  $2.5 \times 10^{-5}$  mole of complex per silver mole. The third solution was added after 4 percent of the silver nitrate solution had been added to the reaction vessel, addition being completed when 74 percent of the silver nitrate had been added to the reaction vessel.

Neutron activation analysis confirmed that approximately 60 percent of the osmium hexacyanide complex in the reaction vessel was incorporated in the silver chloride grains. Table II shows that the presence of the hexacoordinated transition metal complex in the grains resulted in higher sensitivity at comparable levels of fog and contrast.

TABLE II

|    | Emulsion | Speed | Fog  | Contrast |
|----|----------|-------|------|----------|
| 10 | 1        | 100   | 0.06 | 4.2      |
|    | 2        | 180   | 0.05 | 4.0      |

##### Example 4

##### Emulsion 3

0.3  $\mu m$  Undoped  $AgCl$  (Control)

The procedure described above in connection with Emulsion 1 was repeated, except that the emulsion was washed by ultrafiltration and development was accomplished in 12 minutes instead of 5 minutes.

##### Emulsion 4

0.3  $\mu m$   $[Ru(CN)_6]^{-4}$  Doped  $AgCl$

##### (Example)

The procedure described above in connection with Emulsion 3 was repeated, except that the third aqueous solution contained 124 mg of  $K_4Ru(CN)_6$ , which amounts to  $5.0 \times 10^{-5}$  mole per mole of silver in the reaction vessel. Addition of the third solution was completed when 70 percent of the total silver nitrate was added.

Sensitization and coating of the emulsion was similar to that of Emulsion 3. Neutron activation confirmed that approximately 85 percent of the ruthenium complex in the reaction vessel was incorporated in the grains. Table III demonstrates enhancement of speed and contrast.

TABLE III

|    | Emulsion | Speed | Fog  | Contrast |
|----|----------|-------|------|----------|
| 30 | 3        | 100   | 0.07 | 3.4      |
| 35 | 4        | 145   | 0.07 | 3.9      |

##### EXAMPLE 5

##### Emulsion 5

150  $\mu m$ ole  $[Os(CN)_6]^{-4}$  Doped  $AgCl$

##### (Example)

This emulsion was prepared similarly as Emulsion 3, except that the distilled water solution contained 417 mg  $K_4Os(CN)_6$ , which amounts to  $1.5 \times 10^{-4}$  mole per mole of silver.

##### Emulsion 6

0.2  $\mu m$ ole  $[Os(CN)_6]^{-4}$  Doped  $AgCl$

##### (Control)

This emulsion was prepared similarly as Emulsion 3, except that the distilled water solution contained 0.56 mg  $K_4Os(CN)_6$ , which amounts to  $2.0 \times 10^{-7}$  mole per mole of silver.

Portions of Emulsions 3, 4, 5, and 6, were given an optimal sulfur sensitization. The emulsions were then exposed and processed as previously described. The results are summarized in Table IV:

TABLE IV

| Emulsion | Speed | Fog  |
|----------|-------|------|
| 3        | 100   | 0.09 |
| 4        | 162   | 0.14 |
| 5        | 204   | 0.12 |
| 6        | 102   | 0.11 |

Table IV shows that further improved speeds can be obtained when the  $[\text{Os}(\text{CN})_6]^{-4}$  is incorporated in a sulfur sensitized emulsion. However, incorporation of the osmium cyanide coordination complex at concentrations below 1  $\mu\text{mole}$  per silver mole, illustrated by Emulsion 6, did not produce an increase in photographic speed.

#### COMPARATIVE EXAMPLES

Example 5 was repeated, but with  $5.0 \times 10^{-6}$  mole per silver mole of each of the following hexacoordination complexes being substituted for the ruthenium or osmium cyanide complex:



The cobalt and rhodium complexes were both observed to desensitize the emulsion while the iridium complex doped emulsion did not differ significantly in its photographic sensitivity from the undoped control emulsion. While the iron complex decreased fog as compared to the undoped control emulsion, it also reduced speed by 0.2 log E.

To determine the importance of the cyanide ligands, Example 5 was repeated, but an osmium or ruthenium coordination complex lacking a cyanide ligand was substituted. The complex formula with its concentration in micromoles per silver mole shown parenthetically was as follows:



In each instance the emulsion was significantly reduced in speed.

The invention has been described in detail with particular reference to preferred embodiments thereof, but it will be understood that variations and modifications can be effected within the spirit and scope of the invention.

What is claimed is:

1. A photographic silver halide emulsion comprised of radiation sensitive silver halide grains containing greater than 50 mole percent chloride and less than 5 mole percent iodide, based on total silver, with any residual halide being bromide, said grains exhibiting a face centered cubic crystal lattice structure formed in the presence of a hexacoordination complex of rhenium, ruthenium, or osmium with at least four cyanide ligands.

2. A photographic emulsion according to claim 1 further characterized in that said silver halide grains

contain greater than 70 mole percent chloride, based on total silver.

3. A photographic emulsion according to claim 1 further characterized in that said silver halide grains contain less than 2 mole percent iodide, based on total silver.

4. A photographic emulsion according to claim 1 further characterized in that said silver halide grains exhibit gold surface sensitization.

5. A photographic emulsion according to claim 1 further characterized in that said silver halide grains additionally exhibit sulfur surface sensitization.

6. A photographic emulsion according to claim 1 further characterized in that said rhenium, ruthenium, or osmium is present in said emulsion in a concentration of from  $1 \times 10^{-6}$  to  $5 \times 10^{-4}$  mole per silver mole.

7. A photographic emulsion according to claim 1 further characterized in that said hexacoordination complex satisfies the formula:



where

M is rhenium, ruthenium, or osmium,

L is a bridging ligand,

y is the integer zero, 1, or 2, and

n is -2, -3, or -4.

8. A photographic emulsion according to claim 7 further characterized in that L is a halide ligand.

9. A photographic emulsion according to claim 7 further characterized in that y is zero and n is -4.

10. A photographic silver halide emulsion comprised of radiation sensitive silver halide grains surface sensitized with at least one of gold and sulfur, said grains containing greater than 70 mole percent chloride and less than 2 mole percent iodide, based on total silver, with any residual halide being bromide, said grains exhibiting a face centered cubic crystal lattice structure formed in the presence from  $1 \times 10^{-6}$  to  $5 \times 10^{-4}$  mole per silver mole of a hexacoordination complex of the formula:



where

M is ruthenium or osmium,

L is halide, and

y is the integer zero, 1, or 2.

11. A photographic emulsion according to claim 10 further characterized in that said hexacoordination complex is present in a concentration of from  $10^{-5}$  to  $10^{-4}$  mole per silver mole.

12. A photographic emulsion according to claim 10 further characterized in that said silver halide grains are sulfur and gold surface sensitized.

13. A photographic emulsion according to claim 10 further characterized in that said silver halide grains contain greater than 85 mole percent chloride, based on silver.

14. A photographic emulsion according to claim 13 further characterized in that said silver halide grains are silver chloride grains.

\* \* \* \* \*